

Oct. 19, 1937.

G. F. NADEAU

2,096,617

MANUFACTURE OF PHOTOGRAPHIC FILM

Original Filed June 22, 1935 2 Sheets-Sheet 1

Fig.1.



Fig.2.



Fig.3.



Inventors

Gale F. Nadeau,

Newton M. Perrins,

Henry S. Boynton

Attorneys

Oct. 19, 1937.

G. F. NADEAU

2,096,617

MANUFACTURE OF PHOTOGRAPHIC FILM

Original Filed June 22, 1935 2 Sheets-Sheet 2

Fig.4.



Fig.5



Fig.6.



Fig.7.



Fig.8.



Fig.9.



Fig.10.



Inventor:

Gile F. Nadeau,

Warren M. Perrine,

Henry S. Begton

By

Attorneys

## UNITED STATES PATENT OFFICE

2,096,617

## MANUFACTURE OF PHOTOGRAPHIC FILM

Gale F. Nadeau, Rochester, N. Y., assignor, by  
mesne assignments, to Eastman Kodak Com-  
pany, Jersey City, N. J., a corporation of New  
Jersey

Application June 22, 1935, Serial No. 27,916  
Renewed March 30, 1937

18 Claims.

(Cl. 95—9)

This invention relates to photographic mate-  
rials and more particularly to photographic film  
having a high degree of flexibility and satisfac-  
tory emulsion adherence characteristics in which  
5 an improved type of substratum or undercoat is  
employed between the light-sensitive emulsion  
and the film support.

This application is in part a continuation of  
my co-pending application, Serial No. 1547, filed  
10 January 12, 1935.

In the manufacture of photographic film, espe-  
cially film of the so-called safety type, in which  
a light-sensitive emulsion is coated onto a flexible,  
15 relatively uninflammable cellulose derivative  
support, two rather serious problems are en-  
countered. One is to get the emulsion to stick  
properly to the support, and the other is to  
attain the requisite degree of flexibility. When  
20 the adhesion is good, the film as a whole is often  
brittle and will fracture even with moderate  
bending. This is probably due to the fact that,  
since the emulsion adheres so closely to the sup-  
port, it is, broadly speaking, substantially con-  
25 tinuous with it. Accordingly, as soon as the  
emulsion breaks, the energy of impact produced  
by the fracture is transmitted directly to the  
support and causes it to break also. Experience  
has shown that when the emulsion adheres less  
30 tenaciously to the support, the film is often found  
to have unsatisfactory stripping qualities, that is,  
the emulsion can be lifted or stripped from the  
base or support too readily to meet the require-  
ments of many photographic uses. It has ac-  
35 cordingly always been found necessary heretofore  
to effect some sort of compromise between adher-  
ence on the one hand and brittleness on the  
other, and it is well known that one property  
always invariably gained at the expense of the  
other.

40 As is well known, gelatin emulsions (which are  
colloidal solutions or dispersions of gelatin in  
water) cannot be made to adhere directly to a  
cellulose derivative support, because water will  
not wet this type of surface. It is accordingly  
45 necessary to apply to the cellulose derivative sup-  
port a thin layer, substratum, or "sub", as it is  
generally called, of gelatin in order to provide a  
surface to which the emulsion will stick.  
Although a gelatin emulsion, as such, will not  
50 adhere to the support, a gelatin sub can be made  
to adhere if it is applied from a subbing solution  
containing solvents which, not only wet, but  
superficially attack, soften, or swell the cellulose  
derivative material and thus assist in anchoring  
55 the gelatin thereto. Once the gel sub is applied,

it is a relatively simple matter to make the light-  
sensitive aqueous emulsion stick to the support,  
since water will readily wet and soften the sur-  
face of the gel coating and the emulsion can thus  
be made to adhere to it.

5 It should be pointed out that when an emulsion  
is applied to a gel-subbed base, the emulsion and  
gel sub tend to merge and form what, for all  
intents and purposes, may be considered a single  
continuous gelatin layer on the film, and that the  
10 degree of adherence of the emulsion to the sup-  
port is dependent upon the degree of adherence  
of the gel sub to the support or to the intervening  
substrata if any. This adherence of the gel sub  
is controlled in practice by controlling the  
15 "strength" of the gel subbing solution, that is, the  
solvent or softening power of the subbing solution  
on the cellulose derivative material or inter-  
vening substrata. This control of solvent or  
softening power of the solution is accomplished  
20 by regulating the kind or amount of each of the  
solvents used in compounding it. A "strong"  
gel subbing solution is, accordingly, one which  
has a relatively strong solvent, softening or  
swelling action on the support material and  
25 causes the deposited gel sub to adhere tena-  
ciously thereto, while a "weak" subbing solution is  
one which is only weakly solvent with respect to  
the support material and will cause the deposited  
gelatin coating to adhere only slightly. In gen-  
30 eral, it may be said that the stronger the gel sub-  
bing solution, the greater will be the degree of  
adherence of the sub to the support and the  
greater the brittleness of the completed film.

35 The problem of obtaining proper adherence of  
the emulsion without an undue increase in brittleness  
is a difficult one, especially when dealing  
with the so-called safety types of films in which  
the support is formed from a cellulose organic  
derivative, such as cellulose acetate. When em-  
ploying cellulose nitrate as the support, it is pos-  
sible to use a relatively weak gel subbing solution  
and thus, to a certain extent, to keep the adher-  
ence (and consequently brittleness) down to ap-  
proximately the proper value, but with cellulose  
45 organic derivative supports, such as those formed  
of cellulose acetate, or cellulose acetate propio-  
nate, for example, much stronger subbing solu-  
tions must be employed with the result that ex-  
cessive adherence, and therefore excessive brit-  
50 tleness occurs. It has accordingly been neces-  
sary with this latter type of support, first to apply  
a thin cellulose nitrate sub (which can itself be  
subbed with relatively weak subbing solutions),  
and then to apply a gel sub to the nitrate surface,

5

10

15

20

25

30

35

40

45

50

55

followed by the emulsion coating, but this is disadvantageous because of the fact that it introduces a certain amount of cellulose nitrate into the finished film, making it difficult to meet the 5 underwriters' specifications for safety film. Aside from this attempted solution of the problem the question of brittleness (where emulsion adherence was satisfactory) has remained substantially the same, and even films including 10 nitrate undercoats have proved insufficiently free from this defect to meet all of the rigid requirements of cinematographic use.

In an attempt to solve this problem of obtaining proper flexibility without an undue sacrifice of 15 emulsion adherence, it has been proposed to employ an extra heavy cellulose nitrate undercoat underneath the gel sub and, while this expedient does appreciably increase flexibility, without an extra large decrease in adherence, it suffers the 20 disadvantage pointed out above, namely, that it introduces a relatively large amount of cellulose nitrate into the finished product. Many other expedients looking toward the same end have been employed, for example, the use of an undercoat 25 of rubber or similar material, but it has been found that, similarly to cellulose derivative undercoats, the impact arising from rupture of the emulsion is transmitted through the rubber layer, causing it to break, and this break is carried on 30 into the material of the underlying support. Somewhat similar to such products, and suffering many of the same defects, are various laminated structures in which bases consisting of cellulose organic derivatives or other materials have 35 applied thereover a layer or layers of resinous or rubber-like materials of substantial thickness, these layers constituting a material part of the support and being applied, either in the form of separate sheets united to the base by appropriate 40 cement, or deposited, as coatings, from appropriate solutions.

It is the principal object of the present invention to overcome the above-mentioned prior art 45 difficulties and to provide a photographic film having a high degree of flexibility or freedom from brittleness and at the same time satisfactory emulsion adherence. A further object is to provide an improved type of safety film in which flexibility is rendered completely independent of 50 the degree of adherence. A further object is to provide an improved type of safety film in which flexibility is rendered completely independent of the degree of adherence between the emulsion and the underlying substrata. A specific object 55 is to provide a film having a formaldehyde-aryl sulphamide resin sub or undercoat between the light-sensitive gelatin layer and the film base. Other objects will appear hereinafter.

I have found that if the support is first coated 60 with a thin layer consisting essentially of a synthetic resin of the type sold under the trade name "Santolites" which are products obtained by the interaction of formaldehyde or a polymer of formaldehyde with an aryl sulphamide or an alkyl 65 N-substituted aryl sulphamide, almost any strength of gel subbing solution may be employed in the subbing operation and the gelatin emulsion may be bound to the gel sub and other substrata as tightly as desired without giving rise to brittleness in the finished film. In other words, 70 the use of these resins as undercoats renders the matter of flexibility independent of the degree of adherence between the emulsion and the underlying substrata.

In the accompanying drawings, I have illus-

trated in greatly exaggerated section several film structures produced in accordance with my invention, and a test by which the flexibility of such films may be determined.

Figs. 1, 2, and 3 are sections through the body 5 of a photographic film produced in accordance with my invention and including a formaldehyde-aryl sulphamide resin sub.

Figs. 4 and 5 illustrate the manner of carrying 10 out a brittleness test as described herein.

Figs. 6 and 7 illustrate the behaviour of a relatively brittle film when subjected to the test illustrated in Figs. 4 and 5.

Figs. 8, 9, and 10 illustrate the behaviour of a film such as shown in Figs. 1, 2, and 3 respectively, 15 upon being subjected to the test illustrated in Figs. 4 and 5.

In the following examples and description, I have set forth several of the preferred embodiments of my invention, but they are included 20 merely for purposes of illustration and not as a limitation thereof.

After carrying out extensive work with various types of resinous materials, I have found that in 25 order to fulfill the requirements of use as a substratum in the photographic film, the resin must be sufficiently adhesive when dissolved in appropriate solvents to stick properly to the cellulose derivative material of the support, that is, so that the completed film will pass the stripping tests 30 35 herein described. The material must be compatible with the cellulose derivative and must also be compatible with the photographic emulsion in the sense that it shall not fog or reduce the sensitivity thereof or adversely affect any of the various processing steps to which the film is subjected during development. All of these requirements I have found are fulfilled by the formaldehyde-aryl sulphonamide resins.

The particular resins which are used as sub- 40 layers according to my invention are colorless odorless products, soluble in benzene and acetone, obtained by the interaction of formaldehyde or polymers of formaldehyde with an aryl sulphamide or an alkyl N-substituted aryl sulphamide 45 and are manufactured and sold by the Monsanto Chemical Company under the trade name "Santolites". Their preparation is described on pages 177-178 of the text by Scheiber and Sandig entitled "Artificial resins", published in 50 1931 by Isaac Pitman & Sons, Ltd., London, England, and more particularly in German Patents 359,676; 369,644, British Patent 349,956, and U. S. Patents 1,907,554 and 1,908,159. Probably 55 the most typical resin is the product of interaction of paratoluene sulphoethylamide with formaldehyde.

The subbing of the film support with the resin 60 solution may be carried out by any technique well known to those skilled in the art. The material 65 may be conveniently applied to a cellulose acetate support, for example, from a 2% to 10% solution in methyl or ethyl alcohol or acetone, or any other suitable solvent for the resin. After 70 drying, the resin-coated support is coated with a thin protective layer of cellulose nitrate, cellulose acetate, or other cellulose derivative, merely as a matter of convenience in handling the material in subsequent operations. A thin gelatin sub is then applied to the protective cellulose derivative coating in order to form a proper 75 surface upon which to deposit the final coating of emulsion, as previously described. The application of the resin, cellulose derivative and gelatin layers may be accomplished by any of

the well known subbing operations, such as immersion, bead application, or otherwise. The material may be subbed on one or both sides, depending upon the type of film being produced.

5 For example, in the manufacture of portrait film, it is customary to apply a layer of gelatin to the surface opposite the emulsion and in X-ray film to apply gelatin subs and emulsion to both surfaces in order to give greater flatness to the product and for other purposes. In accordance with my invention the support or film base is subbed on both surfaces with the resin in producing this type of product.

15 *Example 1*

In producing a film in accordance with one form of my invention, a support consisting of a sheet or film of cellulose acetate is led through an immersion type hopper containing a 10% 20 methyl or ethyl alcohol solution of a formaldehyde-aryl sulphamide resin of the type herein described at a linear speed of approximately 3 feet per minute. The support is then led through an appropriate drying apparatus maintained at 25 a temperature of approximately 120-200° F., where the solvent is evaporated from the surface of the material and a resin layer of approximately .00008 inch in thickness is deposited thereon. The resin-coated material is then carried 30 through a second immersion type hopper containing a solution of a cellulose derivative say, a 2½% solution of a high alcohol-soluble, low viscosity nitrocellulose dissolved in a solvent comprising 90% of methyl alcohol and 10% of butyl alcohol. Following appropriate drying of the 35 nitro coating, which is also extremely thin (of approximately the same order of thickness as the resin coating), the material is given a third extremely thin coating or sub of gelatin by the 40 immersion or equivalent method, the gelatin solution having approximately the following composition:

| Per cent by weight |      |
|--------------------|------|
| Gelatin            | 1.0  |
| Water              | 10.0 |
| Acetic acid        | 0.5  |
| Methanol           | 88.5 |

The gelatin-coated material is then dried at an appropriate temperature and the usual gelatin-silver halide emulsion coating deposited on the gelatin surface in a well known manner, thus completing the film.

55 *Example 2*

A sheet or film of cellulose acetate propionate of appropriate thickness is coated with an extremely thin layer of a Santolite resin, for example, the product formed by condensing ethyl paratoluene sulphamide with formaldehyde, the 60 resin in this case being deposited from a 7% solution of methyl alcohol. Following appropriate drying of the resin layer as in Example 1, a thin gelatin layer is deposited upon the resin layer from a solution or dispersion having approximately the following composition:

| Per cent by weight |      |
|--------------------|------|
| Gelatin            | 1.0  |
| Acetic acid        | 1.0  |
| H <sub>2</sub> O   | 4.0  |
| Methyl alcohol     | 30.0 |
| Acetone            | 64.0 |

After drying the gelatin layer, the light-sensitive emulsion layer is deposited on the film as before.

65 *Example 3*

A sheet or film of cellulose acetate or cellulose acetate propionate of appropriate thickness is coated with an extremely thin layer comprising 5 a mixture of gelatin and a formaldehyde aryl sulphamide resin, this coating being deposited from a solution having approximately the following composition:

|                                    | Per cent by weight |
|------------------------------------|--------------------|
| Gelatin                            | 1.0                |
| Formaldehyde-aryl sulphamide resin | 1.0                |
| Acetic acid                        | 1.0                |
| Acetone                            | 50.0               |
| Methyl alcohol                     | 43.0               |
| Water                              | 4.0                |

After appropriate drying of the gelatin-resin coating, the emulsion is applied to the resin-subbed surface of the support in the usual manner.

As will be observed from the above examples, various protective layers may be employed over the resin coating, if desired, or the protective layer may be omitted as hereinafter described. I have found that these layers may be composed of cellulose nitrate, cellulose acetate, and, in fact, almost any of the cellulose ester compositions customarily used for film making purposes. Likewise, the material of the support may be composed of any suitable cellulose organic derivative material, such as cellulose acetate, cellulose propionate, cellulose butyrate, or a mixed cellulose organic ester, such as cellulose acetate propionate, cellulose acetate butyrate, cellulose acetate stearate, and the like. Although not limited thereto, my invention relates primarily to the manufacture of the so-called safety types of photographic film in which the support is composed of a relatively non-inflammable material, such as the cellulose organic esters, since it is 40 with this type of material that the problem of brittleness is most severe.

Although in the above examples, I have found it convenient to illustrate my invention by reference to photographic films coated or subbed on one side only, the use of the formaldehyde-aryl sulphamide resins as subs as herein described, may be applied with equal success to products, such as X-ray or portrait film, in which gelatin or emulsion coatings or both are deposited on 50 both surfaces to give greater flatness to the film. It will be apparent that in such products, it is as necessary to prevent brittleness arising from the application of the gelatin on one side of the film as on the other. I have found that brittleness is as effectively prevented by the use of the thin resinous layers in accordance with my invention as in the case of those films which have gelatin layers or coatings on one surface only.

The customary tests by which the properties 60 of my improved type of photographic films are determined will now be described. These are the so-called dry stripping, wet stripping, and brittleness or flexibility tests.

The dry stripping test is carried out as follows: 65 A piece of the complete emulsion-coated film of a convenient size, say, 6 inches wide by 40 inches long, is held at one end with both hands with the emulsion side toward the operator and is then torn lengthwise with successive quick motions of 70 one hand, the tearing generally being carried out at a slight angle to the edge of the strip in order to obtain an oblique tear. The tears thus produced are more or less jagged. An attempt is now made to pull back the emulsion coating from 75

the film with the fingernails and the degree to which the emulsion separates from the support is a measure of its adherence. It will, of course, be understood that the standards of emulsion adherence will vary for different types of film and what is considered satisfactory for one film may not be satisfactory for another. For example, stripping (emulsion adherence) is said to be satisfactory for X-ray film if the emulsion cannot be stripped back more than three or four inches. For Cine film, on the other hand, the stripping should not be greater than about  $\frac{1}{4}$  of an inch.

The wet stripping test is carried out as follows: A strip of the emulsion-coated film of convenient size is soaked in water at 70° F. for ten minutes. It is then removed from the water and fixed on a flat surface with the emulsion side up. The emulsion is then gouged or creased with the fingernails at points near the middle and end of the strip, each nail scratch tearing the emulsion away from the support to a certain extent. The scratched places are then rubbed with considerable force with the balls of the fingertips for several seconds. A film is said to have satisfactory wet stripping (emulsion adherence) properties when no peeling, or substantially no peeling, of the emulsion occurs as a result of this rubbing action. Wet stripping is said to be unsatisfactory when an appreciable or large amount of the emulsion comes off. For most types of film it should not be possible to remove pieces wider than  $\frac{1}{4}$  inch by this test.

The brittleness test is carried out as follows: A strip of film of convenient size is heated for forty-five minutes in a brittleness oven in which air having a controlled relative humidity of 20-25% and a temperature of 110-120° F. is circulated. The film is then removed from the oven and folded at ten different places along the strip by pressing the fold suddenly between the forefinger and the thumb. If the film is brittle, this sudden folding will cause it to break or snap in two at the fold. The flexibility may be defined in terms of freedom from brittleness which may be figured directly in percentages from the results of the test. For example, a film is said to be 60% free from brittleness if it ruptures at only four out of ten folds.

My invention will be further understood by reference to the accompanying drawings. In Fig. 1 I have illustrated a section through a photographic film produced substantially as described in Example 1 in which the letter A designates a cellulose derivative support composed of cellulose acetate, for example. Superimposed on and tightly adhering thereto is an extremely thin undercoat composed of a Santolite (formaldehyde-aryl sulphamide resin), this undercoat being approximately .00008 inch in thickness. B designates a thin protective layer of cellulose nitrate or cellulose acetate, while C is a thin gelatin sub which adheres to the cellulose nitrate or acetate layer B. D is the final gelatino-silver halide emulsion layer which adheres tightly to the gelatin sub C.

Fig. 2 represents a film structure prepared as described in Example 2 and differing from that of Fig. 1 in that the protective layer of cellulose derivative B has been omitted, it being one of the features of the formaldehyde-aryl sulphamide resins that they may be conveniently handled without a protective coating due to the fact that they are not tacky at ordinary temperatures or the temperatures customarily met with in film manufacture.

Fig. 3 represents a film structure similar to that of Fig. 2 except that the gelatin layer or sub has been omitted and a single layer X composed of a mixture of gelatin and a formaldehyde-aryl sulphamide resin has been deposited upon the support and the emulsion layer D laid down directly upon this gelatin-resin layer.

Figs. 4 and 5 illustrate graphically the manner of carrying out the brittleness test above referred to. The film F, after removal from the brittleness oven, is folded at a given place into the form of a short loop, the gelatin layer D being outermost. This loop is then closed by means of the forefinger and thumb. The pressure being applied as suddenly as possible and in the direction indicated by the arrows in Fig. 5.

In Figs. 6 and 7 there are illustrated the results obtained when an ordinary type of photographic film comprising—a support A, a thin cellulose derivative undercoat, and the emulsion layer D over the gel sub—is subjected to the test. It will be seen that the crack starting in the emulsion penetrates through the layers B and C and goes on into the material of the support. This crack almost invariably continues on through the support with the result shown in Fig. 7. The film here illustrated is a typical prior art product and one from which the resinous sub or undercoat of the present invention is absent. This product is also one in which there is a high degree of adherence between the emulsion and the gel sub layer and between these layers and the underlying cellulose derivative material.

Fig. 8 illustrates the results obtained when a film employing the resinous subs or undercoats of my invention is subjected to the test illustrated in Figs. 4 and 5. This film is in all respects the same as that illustrated in Figs. 6 and 7 except that a layer X of a Santolite (formaldehyde-aryl sulphamide resin) has been applied to the support before application of the cellulose derivative layer B, the gel sub C, and the emulsion coating D. The emulsion is made to adhere to the support with the same degree of tenacity, as in the product illustrated in Figs. 6 and 7, but the product of Fig. 8 differs from that of Fig. 6 in the fact that, although the crack starting in the emulsion may continue through the gel sub, the cellulose derivative sub and even the resin layer itself, it does not in any case, penetrate into the support itself.

Figs. 9 and 10 illustrate graphically the results obtained in subjecting the film structures of Figs. 2 and 3, respectively, to the test illustrated in Figs. 4 and 5. In the structure of Fig. 2 the crack starting in the emulsion layer penetrates the gelatin and resin sub-layers but does not penetrate the support itself. A similar result is obtained with the product of Fig. 3 as illustrated in Fig. 10.

Figs. 8, 9, and 10 strikingly illustrate the fact that a photographic film produced in accordance with my invention is characterized by the unusual property of 100% freedom from brittleness or, in other words, it has 100% flexibility. In addition to this remarkable property, films produced in accordance with my invention respond satisfactorily to both the wet and dry stripping tests above described. In this connection, it should be pointed out that one of the outstanding features of my invention is the fact that the adherence of the emulsion may be regulated without regard to the flexibility of the film. In other words, it is possible to produce a film in which the emulsion adheres to the support with the highest practicable degree of tenacity without inducing any

brittleness whatever in the film as a whole or causing the support material to break on bending, either during cinematographic or other use, or when subjected to the tests herein described.

5 While I offer no particular explanation or theory to account for the unusual results obtained in the practice of my invention, it is evident that the resinous subs or undercoats herein described offer some means of dissipating the impact of the rupturing emulsion. This effect is to be distinguished from the mere cushioning effect characteristic of elastic or semi-elastic materials. In many, although not all, cases, the break occurring in the emulsion will penetrate even the lowermost resinous layer, and these layers may even be released from the support, to a slight extent, but in no case does the break penetrate the material of the support itself.

In the above description and in the claims I have used the terms "substratum", "sub layer", or "sub", "subbing", "undercoat", etc. By a substratum, sub layer or sub I refer broadly to any layer, whether composed of a single layer or a plurality of layers, employed between the emulsion and the film base. The term "undercoat" refers to a single layer used underneath any other layer except the emulsion. It is customary, however, in the case of a plurality of layers underneath the emulsion to refer to the layer next to the emulsion as a sub and the underlying layers as undercoats. The term snubbing is employed broadly to indicate the application of a thin layer of a material to the surface of a film, whether previously coated or not.

35 Furthermore, by the term "sub" I refer to extremely thin layers or undercoats of material of the order of only a few millionths of an inch in thickness, such, for example, as the resin layer of Example 1. Inasmuch as the thickness of these layers is of this extremely small order of magnitude, it is evident that it may vary by a number of millionths, either above or below the preferred thickness of .00008 inch. It will also be evident that the thickness of these subs will 45 vary in accordance with the usual variations met with in the type of film base used. The thicker types of film base tolerate a slightly thicker sub, although in no case is the thickness sufficient to be regarded as a lamination in the ordinary sense 50 of the word as in those cases where a laminated film base is built up by the superimposition of a number of layers of appreciable or relatively substantial thickness.

What I claim is:

55 1. A photographic film of satisfactory flexibility and free from brittleness, comprising a cellulose organic derivative support and a photographically sensitive colloid layer adhesively joined to the support by a composite intervening layer comprising an extremely thin sub composed of a resin formed by the condensation of formaldehyde or polymers of formaldehyde with a member of the group consisting of the aryl sulphamids and the alkyl N-substituted aryl sulphamids adhesively 60 joined to the support, a cellulose derivative sub adhesively joined to the resin sub and a gel sub adhesively joined to the cellulose derivative sub and to the sensitive colloid layer, said intervening layer rendering the flexibility characteristics of the film as a whole independent of the degree of adhesion existing between the photographically sensitive layer and the subbed support.

2. A photographic film of satisfactory flexibility and free from brittleness, comprising a cellulose organic derivative support and a photo-

graphically sensitive colloid layer adhesively joined to the support by a composite intervening layer comprising an extremely thin sub composed of a resin formed by the condensation of formaldehyde or polymers of formaldehyde with 5 an alkyl N-substituted aryl sulphamid, adhesively joined to the support, a cellulose derivative sub adhesively joined to the resin sub and a gel sub adhesively joined to the cellulose derivative sub and to the sensitive colloid layer, said 10 intervening layer rendering the flexibility characteristics of the film as a whole independent of the degree of adhesion existing between the photographically sensitive layer and the subbed support.

3. A photographic film of satisfactory flexibility and free from brittleness, comprising a cellulose organic derivative support and a photographically sensitive colloid layer adhesively joined to the support by a composite intervening 20 layer comprising an extremely thin sub composed of a resin formed by the condensation of formaldehyde or polymers of formaldehyde with ethyl paratoluene sulphamid adhesively joined to the support, a cellulose derivative sub adhesively joined to the resin sub and a gel sub adhesively joined to the cellulose derivative sub and to the sensitive colloid layer, said intervening 25 layer rendering the flexibility characteristics of the film as a whole independent of the degree 30 of adhesion existing between the photographically sensitive layer and the subbed support.

4. A photographic film of satisfactory flexibility and free from brittleness, comprising a cellulose organic acid ester support and a photographically sensitive colloid layer adhesively joined to the support by a composite intervening 35 layer comprising an extremely thin sub composed of a resin formed by the condensation of formaldehyde or polymers of formaldehyde with 40 a member of the group consisting of the aryl sulphamids and the alkyl N-substituted aryl sulphamids adhesively joined to the support, a cellulose derivative sub adhesively joined to the resin sub and a gel sub adhesively joined to the cellulose derivative sub and to the sensitive colloid layer, said intervening 45 layer rendering the flexibility characteristics of the film as a whole independent of the degree of adhesion existing between the photographically sensitive layer and 50 the subbed support.

5. A photographic film of satisfactory flexibility and free from brittleness, comprising a cellulose organic acid ester support and a photographically sensitive colloid layer adhesively joined to the support by a composite intervening layer comprising an extremely thin sub composed of a resin formed by the condensation of formaldehyde or polymers of formaldehyde with an alkyl N-substituted aryl sulphamid, adhesively joined to the support, a cellulose derivative sub adhesively joined to the resin sub and a gel sub adhesively joined to the cellulose derivative sub and to the sensitive colloid layer, said intervening layer rendering the flexibility characteristics of the film as a whole independent of the degree of adhesion existing between the photographically sensitive layer and the subbed support.

6. A photographic film of satisfactory flexibility and free from brittleness, comprising a cellulose organic acid ester support and a photographically sensitive colloid layer adhesively joined to the support by a composite intervening

layer comprising an extremely thin sub composed of a resin formed by the condensation of formaldehyde with ethyl paratoluene sulphamid adhesively joined to the support, a cellulose derivative sub adhesively joined to the resin sub and a gel sub adhesively joined to the cellulose derivative sub and to the sensitive colloid layer, said intervening layer rendering the flexibility characteristics of the film as a whole independent of the degree of adhesion existing between the photographically sensitive layer and the subbed support.

7. A photographic film of satisfactory flexibility and free from brittleness comprising a cellulose acetate support and a photographically sensitive colloid layer adhesively joined to the support by a composite intervening layer comprising an extremely thin sub composed of a resin formed by the condensation of formaldehyde or polymers of formaldehyde with a member of the group consisting of the aryl sulphamids and the alkyl N-substituted aryl sulphamids adhesively joined to the support, a cellulose nitrate sub adhesively joined to the resin sub and a gel sub adhesively joined to the cellulose derivative sub and to the sensitive colloid layer, said intervening layer rendering the flexibility characteristics of the film as a whole independent of the degree of adhesion existing between the photographically sensitive layer and the subbed support.

8. A photographic film of satisfactory flexibility and free from brittleness comprising a cellulose acetate support and a photographically sensitive colloid layer adhesively joined to the support by a composite intervening layer comprising an extremely thin sub composed of a resin formed by the condensation of formaldehyde or polymers of formaldehyde with an alkyl N-substituted aryl sulphamid, adhesively joined to the support, a cellulose nitrate sub adhesively joined to the resin sub and a gel sub adhesively joined to the cellulose nitrate sub and to the sensitive colloid layer, said intervening layer rendering the flexibility characteristics of the film as a whole independent of the degree of adhesion existing between the photographically sensitive layer and the subbed support.

9. A photographic film of satisfactory flexibility and free from brittleness comprising a cellulose acetate support and a photographically sensitive colloid layer adhesively joined to the support by a composite intervening layer comprising an extremely thin sub composed of the product of condensation of formaldehyde with ethyl paratoluene sulphamid adhesively joined to the support, a cellulose nitrate sub adhesively joined to the resin sub and a gel sub adhesively joined to the cellulose nitrate sub and to the sensitive colloid layer, said intervening layer rendering the flexibility characteristics of the film as a whole independent of the degree of adhesion existing between the photographically sensitive layer and the subbed support.

10. A photographic film of satisfactory flexibility and free from brittleness, comprising a cellulose organic acid ester support and a photographically sensitive colloid layer adhesively joined to the support by a composite intervening layer comprising an extremely thin sub composed of a resin formed by the condensation of formaldehyde or polymers of formaldehyde with a member of the group consisting of the aryl sulphamids and the alkyl N-substituted aryl sulphamids adhesively joined to the support and a

gel sub adhesively joined to the resin sub and to the sensitive colloid layer, said intervening layer rendering the flexibility characteristics of the film as a whole independent of the degree of adhesion existing between the photographically sensitive layer and the subbed support.

11. A photographic film of satisfactory flexibility and free from brittleness, comprising a cellulose organic acid ester support and a photographically sensitive colloid layer adhesively joined to the support by a composite intervening layer comprising an extremely thin sub composed of a resin formed by the condensation of formaldehyde or polymers of formaldehyde with an alkyl N-substituted aryl sulphamid adhesively joined to the support and a gel sub adhesively joined to the resin sub and to the sensitive colloid layer, said intervening layer rendering the flexibility characteristics of the film as a whole independent of the degree of adhesion existing between the photographically sensitive layer and the subbed support.

12. A photographic film of satisfactory flexibility and free from brittleness comprising a cellulose organic acid ester support and a photographically sensitive colloid layer adhesively joined to the support by a mixed gelatin-resin sub, the resin component of which is composed of the product of condensation of formaldehyde or polymers of formaldehyde with a member of the group consisting of the aryl sulphamids and the alkyl N-substituted aryl sulphamids.

13. A photographic film of satisfactory flexibility and free from brittleness comprising a cellulose organic acid ester support and a photographically sensitive colloid layer adhesively joined to the support by a mixed gelatin-resin sub, the resin component of which is composed of the product of condensation of formaldehyde or polymers of formaldehyde with an alkyl N-substituted aryl sulphamid.

14. A photographic film of satisfactory flexibility and free from brittleness comprising a cellulose organic acid ester support and a photographically sensitive colloid layer adhesively joined to the support by a mixed gelatin-resin sub, the resin component of which is composed of the product of condensation of formaldehyde with ethyl paratoluene sulphamid.

15. A flexible photographic film comprising a cellulose organic derivative support layer, which layer, if uncoated, would be flexible under dry conditions, a photographic colloid layer carried by the support and having the characteristic of becoming brittle in conditions under which the support remains flexible, and a sub layer between the photographic layer and the support layer and adjacent the support layer, all the said layers being strongly adherent one to another, the sub layer comprising a formaldehyde-aryl sulphamide resin and rendering the film permanently highly flexible.

16. A flexible photographic film comprising a cellulose organic derivative support layer, which layer, if uncoated, would be flexible under dry conditions, a photographic colloid layer carried by the support and having the characteristic of becoming brittle in conditions under which the support remains flexible, and a sub layer between the photographic layer and the support layer and adjacent the support layer, all the said layers being strongly adherent one to another, the sub layer comprising the product of condensation of ethyl paratoluene sulphamide with form-

aldehyde and rendering the film permanently highly flexible.

17. A photographic film of high flexibility and free from brittleness, comprising a cellulose organic derivative support and a photographically sensitive colloid layer adhesively joined to the support by a composite intervening layer comprising a thin formaldehyde-aryl sulphamide resin sub adhesively joined to the support and a gel sub adhesively joined to the resin sub and to the sensitive colloid layer, said intervening layer rendering the flexibility characteristics of the film as a whole independent of the degree of adhesion existing between the photographically sensitive layer and the subbed support.

18. A photographic film of high flexibility and

free from brittleness, comprising a cellulose organic acid ester support and a photographically sensitive colloid layer adhesively joined to the support by a composite intervening layer comprising a thin resin sub composed of the product of condensation of ethyl paratoluene sulphamide with formaldehyde and adhesively joined to the support and a gel sub adhesively joined to the resin sub and to the sensitive colloid layer, said intervening layer rendering the flexibility characteristics of the film as a whole independent of the degree of adhesion existing between the photographically sensitive layer and the subbed support.

GALE F. NADEAU. 15